

# UNITED STATES PATENT OFFICE.

HENRY PETRIE FLETCHER, OF FOREST LODGE, NEAR SYDNEY, NEW SOUTH WALES,  
AUSTRALIA.

## PROCESS FOR THE CONVERSION OF WATER PASTES INTO OIL PASTES.

1,317,784.

Specification of Letters Patent.

Patented Oct. 7, 1919.

No Drawing.

Application filed October 17, 1918. Serial No. 258,644.

*To all whom it may concern:*

Be it known that I, HENRY PETRIE FLETCHER, a subject of the King of Great Britain, residing at 64 Arundel street, Forest Lodge, near Sydney, in the State of New South Wales, Australia, have invented certain new and useful Improvements in Processes for the Conversion of Water Pastes into Oil Pastes, of which the following is a specification.

This invention relates to improvements in the manufacture of oil pastes and has been devised in order that the water in a water paste may be removed therefrom and oil substituted for the said water without necessitating an intermediate drying operation and to obtain a satisfactory commercial product.

In the production of certain oil pastes such as that wherein white lead is the base, the material under treatment assumes at one stage of manufacture the form of a wet pulp from which (according to the processes heretofore generally used) it is necessary to remove the water and to thereafter permeate the material with oil.

The salient feature of this invention resides in the provision of chemical and mechanical means whereby the pulp is permeated with oil to form an oil paste and the contained water is expelled without necessitating a distinct drying operation.

The wet pulp which is required to be converted into an oil paste is first treated by the addition of a predetermined quantity of borate of manganese. The proportion of borate of manganese to wet pulp would vary within certain limits hereinafter clearly defined according to the percentage of water contained in the pulp, the quantity of oil required to be incorporated, and the time available for mixing. When treating thick pastes, that is pulp having a comparatively low water content the proportion of borate of manganese added should be small, and when there are to be treated slush pastes that is those having a comparatively high water content the proportion of borate of manganese should be relatively higher.

The preferred proportion for pulp having a water content of approximately 20% by weight is 9 grains of borate of manganese to one pound of wet pulp, which corresponds to approximately  $\frac{1}{8}$  of one per cent.

For slush pastes the proportion may be

progressively raised according to the water content to a maximum for most purposes of twenty-five grains to the pound of wet pulp. Under no circumstances should the proportion of borate of manganese to wet pulp exceed one-half of one per cent. otherwise the desired effect will not be attained in a satisfactory commercial manner, as an excess of borate of manganese in the pulp will saponify the paste.

After the treatment above described a required quantity of oil is added to the pulp and the mass is subjected to mechanical working and mixing, the water being expelled from the pulp and the oil combining therewith. This working or mixing is continued until the oil paste is of the required consistency.

For the purpose of carrying out the working and mixing operation on a commercial scale any ordinary mechanical device or machine known in the art and found suitable may be employed.

Instead of using borate of manganese as hereinbefore described, borax or other boracic acid salts may be employed, though a slightly higher proportion of such substance is necessary.

In the example of wet pulp to be treated, I have mentioned white lead as an example, but the invention is not confined thereto.

What I do claim is:—

1. A process for the conversion of water pastes into oil pastes characterized by the treatment of wet pulp by the addition of boracic acid salts and the mechanical working of the resulting mass with a required quantity of oil.

2. A process for the conversion of water pastes into oil pastes characterized by the treatment of wet pulp by the addition thereto of borate of manganese and the mechanical working of the resulting mass with a required quantity of oil.

3. A process for the conversion of water pastes into oil pastes characterized by the chemical treatment of wet pulp by the addition thereto of not exceeding one-half per cent. by weight, of borate of manganese and the mechanical working and mixing of the resulting mass with a required quantity of oil.

4. A process for the conversion of water pastes into oil pastes wherein a wet pulp is subjected to the action of borate of man-

ganese, said borate of manganese being added in the proportion by weight of not exceeding one-half per cent.

5. A process which comprises adding to a pulp of white lead carrying about 20% of water, an amount of borate of manganese equal to between the approximate limits of one-eighth per cent. to one half per cent., relative to the weight of said pulp.
- 10 6. The herein described process which

comprises mixing a pulp of white lead with a small amount of a borate, then adding oil and working the mass.

In testimony whereof I affix my signature in presence of two witnesses.

HENRY PETRIE FLETCHER.

Witnesses:

M. STARPELL,  
R. BOULTON.